

## UNITED STATES PATENT OFFICE

2,472,335

## METHOD OF FLAMEPROOFING COMBUSTIBLE CELLULOSIC MATERIAL

Andrew McLean, West Kilbride, and Stanley Frederic Marrian, Ardrossan, Scotland, assignors to Imperial Chemical Industries Limited, a corporation of Great Britain

No Drawing. Application November 15, 1945, Serial No. 628,994. In Great Britain January 10, 1945

6 Claims. (Cl. 117—137)

1

The present invention relates to a new or improved method of flame-proofing combustible cellulosic materials that enables them to be washed or laundered in hot aqueous media without losing their flame-proof qualities, and to the resulting flame-proofed cellulosic materials. The invention also relates to a new reagent for use as a flame-proofing component according to the aforesaid new or improved method of flame-proofing combustible cellulosic materials.

Amongst the cellulosic materials to which the invention is especially applicable are textile fabrics, for instance woven or pleated fabrics, threads, yarns, filaments, and fibres, made of cotton, linen, regenerated cellulose, jute, cellulose acetate, and the like.

Various proposals have already been made in connection with the flame-proofing of combustible materials but these proposals for the most part have suffered from such disadvantages as the necessity of having to employ large amounts of reagent to ensure effective flame-proofing thereby stiffening the materials to an undesirable extent, the difficulty experienced in fixing the reagent satisfactorily to the combustible materials so that it will resist laundering operations, and the scarcity or difficulty of production of some of the reagents proposed.

A process has already been disclosed which comprises treating with an acidic-fire-retardant as for example phosphoric acid or calcium phosphate a cellulosic material impregnated with polyethylenimine.

An object of the present invention is to provide a method of flame-proofing combustible cellulosic materials, and a new flame-proofing component used in carrying out the method, yielding flame-proof products that retain their flame-proof qualities subsequent to hot water washing and laundering with hot soap solutions in a more satisfactory degree than heretofore.

It has been found that compositions comprising the novel compound pentaerythritol tetra-orthophosphate can be readily anchored to cellulosic materials impregnated with a polyethylenimine to give flame-proof cellulosic materials which retain their flame-proof characteristics subsequent to their treatment with soap and water washing.

According to the present invention therefore the method of flame-proofing combustible cellulosic materials comprises treating the said materials impregnated with a polyethylenimine with a solution comprising pentaerythritol tetra-orthophosphate.

2

The flame-proofing component according to the present invention for flame-proofing combustible cellulosic materials previously subjected to the action of a polyethylenimine comprises pentaerythritol tetra-orthophosphate.

Crude pentaerythritol tetra-orthophosphate was prepared from pentaerythritol, ortho-phosphoric acid and phosphorus pentoxide as follows, the quantities employed being based upon the molecular ratio of three parts pentaerythritol, four parts of ortho-phosphoric acid and four parts phosphorus pentoxide.

Phosphoric acid (11 gr. of 88%) was added gradually to phosphorus pentoxide (25 gr.) and 15 when the mixture was cool, pentaerythritol (15.3 gr.) was added thereto, the whole being well stirred. The mixture was heated in an oil bath at 120–130° C. for 20 hours with exclusion of moisture and occasional stirring. The crude 20 pentaerythritol tetra-orthophosphate product thus formed probably contained phosphoric acid and pentaerythritol tri-, di- and mono-orthophosphate in addition to the pentaerythritol tetra-orthophosphate.

25 Comparative experiments were carried out to illustrate the differences in behaviour to washing with soap and water of cotton cloth in every case first treated with an aqueous solution of polyethylenimine in the manner specified and subsequently with aqueous solutions of the crude pentaerythritol tetra-orthophosphate, an aqueous solution of a mixture of the three reactants upon which the heat treatment was omitted, the mixture being immediately dissolved in water, 30 and an aqueous solution diluted as required of a mixture of phosphoric acid and phosphorus pentoxide only which were heated together before dissolving in water. Solutions of various concentrations were used.

35 40 Experiments were also carried out to see how to improve the handle or feel of the combustible cellulosic materials and yet retain the desired fireproof qualities after soap and water washing.

The handle or feel is found to be often improved by cutting down the quantity of polyethylenimine with which the combustible cellulosic materials is impregnated, as for example by working with polyethylenimine solutions of strengths lower than 8–12 per cent, but to make 45 certain that in such cases the product remains flame-proof after soap and water washing it is often necessary to treat it subsequent to the pentaerythritol tetra-orthophosphate treatment with an acidified aqueous solution of hexamethoxymethyl melamine or triethoxymethyl 50 55

melamine followed by baking at about 100° C. The said acidification can be effected for example with paratoluene sulphonic acid.

A piece of cotton cloth (12 sq. ins.) was soaked in 10 ml. of a boiling aqueous solution of polyethylenimine for one hour, wrung out and baked in a steam oven overnight. The cloth was then steeped in 15 ml. of an aqueous solution of the crude pentaerythritol tetra-orthophosphate for one hour at room temperature, thoroughly rinsed, and dried. The time given for each operation and the quantities used were arbitrarily fixed.

Testing of flame-proofness was carried out by holding the cloth in a Bunsen flame for 5-10 seconds. Some charring always took place, but if burning was not propagated with any speed in the flame and ceased without afterglow when the cloth was removed from the flame, the cloth was recorded as "flame-proof." If either of these conditions was not satisfied the sample was recorded as "not flame-proof."

The stability of the flame-proofness to washing was tested as follows: The test piece was stirred with 200 ml. water at 40-50° C. for 30 minutes and dried. Flame-proofness was then tested as above. The same piece was then stirred with 200 ml. of 0.25 per cent soap solution at 40-50° C. for 30 minutes, wrung out, rinsed thoroughly in 3 changes of water and dried. The flame-proofness was again tested.

The results obtained are given in the following table:

5 impregnated with an aqueous 8% to 12% polyethylenimine solution.

3. A method as claimed in claim 1 wherein the cellulosic materials are subsequently treated with an acidified aqueous solution of a compound from the group consisting of hexamethoxymethyl melamine and triethoxymethyl melamine, followed by baking at about 100° C.

4. A method as claimed in claim 3 wherein the compound selected is hexamethoxymethyl melamine.

5. A method as claimed in claim 3 wherein the compound selected is triethoxymethyl melamine.

6. Flame-proofed combustible cellulosic textile materials impregnated with polyethylenimine and containing pentaerythritol tetra-orthophosphate as the flameproofing component.

ANDREW MCLEAN.

STANLEY FREDERIC MARRIAN.

#### REFERENCES CITED

The following references are of record in the file of this patent:

#### UNITED STATES PATENTS

| Number    | Name                  | Date          |
|-----------|-----------------------|---------------|
| 1,660,651 | Marshall et al. ----- | Feb. 28, 1928 |
| 2,071,353 | Morgan -----          | Feb. 23, 1937 |
| 2,286,726 | Gordon -----          | June 16, 1942 |

#### FOREIGN PATENTS

| Number  | Country             | Date          |
|---------|---------------------|---------------|
| 476,043 | Great Britain ----- | Apr. 27, 1936 |

| Treatment of Cloth                                                                                                                                                                                                                     | Before<br>Washing | After Water<br>Washing | After Soap and<br>Water Washing |
|----------------------------------------------------------------------------------------------------------------------------------------------------------------------------------------------------------------------------------------|-------------------|------------------------|---------------------------------|
| 10% polyethylenimine, 10% p. t. p. -----                                                                                                                                                                                               | Flameproof.       | Flameproof.            | Flameproof.                     |
| 10% polyethylenimine, 10% control <sup>1</sup> liquor.                                                                                                                                                                                 | do.               | do.                    | not flameproof.                 |
| 10% polyethylenimine, 10% control <sup>2</sup> liquor.                                                                                                                                                                                 | do.               | do.                    | Do.                             |
| 10% polyethylenimine, 10% phosphoric acid.                                                                                                                                                                                             | do.               | do.                    | Do.                             |
| 8% polyethylenimine, 8% p. t. p.                                                                                                                                                                                                       | do.               | do.                    | flameproof.                     |
| 8% polyethylenimine, 8% phosphoric acid.                                                                                                                                                                                               | do.               | do.                    | not flameproof.                 |
| 4% polyethylenimine, 4% p. t. p.                                                                                                                                                                                                       | do.               | do.                    | Do.                             |
| 4% polyethylenimine, 4% phosphoric acid.                                                                                                                                                                                               | do.               | do.                    | Do.                             |
| 5% polyethylenimine, 10% p. t. p.                                                                                                                                                                                                      | do.               | do.                    | Do.                             |
| 5% polyethylenimine, 10% p. t. p. Final treatment with a solution containing 2 grams hexamethoxymethyl melamine+0.05 grams p. toluene sulphonic acid in 18 cc. water (for 12 sq. ins. cloth) followed by baking at 100° C. for 1 hour. | do.               | do.                    | flameproof.                     |
| 5% polyethylenimine, 10% p. t. p. Final treatment with a solution containing 2 gms. triethoxymethyl melamine+0.05 gm. p. toluene sulphonic acid in 18 cc. water (for 12 sq. ins. cloth) followed by baking at 100° for 1 hour.         | do.               | do.                    | Do.                             |

p. t. p.=pentaerythritol tetra-orthophosphate.

<sup>1</sup> Solution of unheated mixture of pentaerythritol, phosphoric acid and phosphorus pentoxide.

<sup>2</sup> Solution of heated mixture of phosphoric acid and phosphorus pentoxide.

We claim:

1. A method of flameproofing combustible cellulosic textile materials which comprises saturating said material impregnated with a polyethylenimine with an aqueous solution comprising 4% to 10% pentaerythritol tetra-orthophosphate, and thereafter drying said material.

2. A method as claimed in claim 1 wherein the cellulosic materials used for treatment with the pentaerythritol tetra-orthophosphate have been

#### OTHER REFERENCES

55 Englund: "Jour. fur prakt. Chem.," Neue folge, vol. 124, pp. 206-7 (1930).

Hassel et al.: "Chem. Abstracts," vol. 32, p. 2801 (1938).

Govaert et al.: "Chem. Abstracts," vol. 38, p. 5201 (1944).